

April 29, 1930.

J. F. WENTZ

1,756,319

CONDUCTOR

Filed March 9, 1925

Fig. 1



Fig. 2



Inventor:  
Jesse F. Wentz,  
by P.W. Adams Atty

## UNITED STATES PATENT OFFICE

JESSE F. WENTZ, OF NEW YORK, N. Y., ASSIGNOR, BY MESNE ASSIGNMENTS, TO  
WESTERN ELECTRIC COMPANY, INCORPORATED, A CORPORATION OF NEW YORK

## CONDUCTOR

Application filed March 9, 1925. Serial No. 13,943.

This invention relates to conductors for the transmission of electrical energy and more particularly to signaling conductors having an external layer of a material of high permeability for the purpose of increasing the inductance of the conductor.

One manner of increasing the inductance of the conductor employed for the transmission of alternating current is to wrap the conductor spirally with a layer of wire or tape of magnetic material. This method is known in the art as continuous inductive loading as distinguished from lump loading by means of inductance coils distributed at intervals along the conductor. Until recently iron has been considered to be the only material suitable for continuous loading but it has now been discovered that a more suitable material may be procured in the form of an alloy of nickel and iron. When these two metals are combined in the proper proportions and the resulting alloy is given a proper heat treatment, a material having a very high permeability at low magnetizing forces is obtained.

One form of this material which has been used in a submarine cable comprises 78½% nickel and 21½% iron. Alloys of nickel and iron having similar characteristics, especially high permeability at low magnetizing forces, have been styled "permalloy". Other properties possessed by these alloys which increase their value as a loading material are a hysteresis loss lower than that of iron and a high resistivity, both properties being conductive to increasing the efficiency of the cable by lowering the effective resistance of the conductor. When it was attempted to employ this material in the form of a tape for continuous loading, difficulties were encountered. It was found that if the permalloy tape was first heated and then cooled before applying to the conductor, internal stresses were set up upon bending of the tape, causing the permeability to be very materially lowered. This difficulty was overcome by applying the tape to the conductor before giving the tape the heat treatment and then subjecting the taped conductor to the heating and cooling necessary to produce high permeability in the loading material.

Further difficulty, however, was experienced in that the permeability of the loading material was lowered by what appeared to be adhesion between the copper conductor and the loading tape. It is believed that this adhesion occurs when the taped conductor is subjected to the high temperatures necessary for the proper heat treatment and that upon subsequent cooling the tape is subjected to stresses which cause a lowering of its permeability.

In the construction of a loaded conductor it was the practice to wrap a layer of magnetic material comprising a nickel-iron alloy closely around the conductor consisting of a central copper wire surrounded by six flat copper strands, the whole making a compact structure with very little space not occupied by metal. To give the loading material the desired magnetic characteristics, this conductor was heated to approximately 850° C. and then cooled at a preferred rate. On heating, both metals expand but the copper, because of its higher temperature coefficient, expands more than the loading material with the result that it presses tightly against the loading material when the conductor is at the high temperature and if the structure is a fairly tight one, the magnetic tape is stretched, an elongation of as much as 1% having been observed. This stretching however, has apparently no direct effect on the magnetic properties since it occurs at a temperature above the magnetic transformation point but it does show effects of high pressure between the metals. At the temperature of 850° C. both metals are relatively soft and since they are forced together by thermal expansion there is a tendency for the loading material to weld to the copper, the extent to which the metals are welded depending on several factors such as the tightness of the copper structure and the character of the metal surfaces. In this connection it has been noted that although the loading material welds to the copper, welding of the copper strands to the central wire has been very rarely observed and no welding has been observed between layers of the loading material when more than one layer has been used. These results suggest that welding is possibly not a simple case of fusion of the two metals.

but some effect brought about by chemical action.

On cooling, the copper conductor contracts more than the magnetic tape. No doubt some of the welds which have been formed break loose when this contraction occurs but the stronger ones hold with the result that the magnetic tape is at points pulled down with the copper and parts of it are bent, stretched or compressed depending upon the particular 10 accidental conditions of adherence. Even though the forces involved may be very small, the stresses at points in the tape may be of considerable magnitude giving strain sufficient to reduce the permeability at spots to a very small fraction of that which the tape would have had if not subjected to such strain. The resultant conductor, therefore, is one which although it may have fairly uniform 15 inductance as measured from foot to foot is loaded with a material which varies in permeability over a wide range in points separated by a fraction of an inch.

The copper tapes upon being stranded 25 about the central conductor do not present a true cylindrical surface since the edges of the strands do not lie in close contact with the central conductor but present spiralled edges. As the cooling proceeds, therefore a 30 sticking or welding of the material may occur at various points along these edges and the subsequent contraction of the copper set up stresses in the alloy tape.

During the cooling portion of the heat 35 treatment the alloy tape may cool more rapidly at first than does the copper conductor due to its intimate contact with the cooling medium so that the alloy tape quickly comes into intimate contact with the copper strands.

Whatever may be the true explanation for 40 the difficulty experienced, it has largely been overcome by providing a small air space between the layer of loading material and the signaling conductor when the loading material is applied. This method of obtaining 45 high permeability is described at length in patent to G. W. Elmen, No. 1,586,887, granted June 1, 1926.

Instead of providing an air space between 50 the conductor and the tape, as the latter is wound in position, the desired result may be obtained by placing a layer of paper upon the conductor before the loading material is wound thereon. This layer of paper is burned 55 out during the subsequent heat treatment thus giving the desired spacing between the loading material and the conductor. This method is described in detail in patent to W. B. Ten Eyck, No. 1,586,862, granted June 1, 1926.

An object of the present invention is to 60 provide for the practical loading of a signaling conductor with a magnetic material which requires heat treatment and whose characteristics are subject to undesired 65 change under applied stresses.

Another object of the invention is to provide a method of applying magnetic loading material to an electrical conductor in such a manner as to prevent the setting up of deleterious stresses in the magnetic material during the subsequent heat treatment. 70

To accomplish these objects, the invention contemplates an electrical conductor, upon which is applied loading material capable of possessing high permeability, and the method of applying this material to the conductor in such a way as to avoid obtaining low or variable values of permeability. This invention is in the nature of an alternative to that disclosed in a copending application of O. E. 80 Buckley, Serial No. 758,984, filed December 31, 1924, and to the above mentioned patents of G. W. Elmen and W. B. Ten Eyck. Each of these inventions has certain advantages over the others, as will be apparent from a 85 consideration of the application and patents mentioned above.

The invention may be more clearly understood by reference to the accompanying drawing, in which Fig. 1 is a view of a loaded 90 conductor embodying the features of the invention, certain portions of the conductor being shown cut away to more clearly disclose the structure; and Fig. 2 is a view showing a simple type of apparatus which may be 95 used for applying the heat treatment to the conductor.

Referring to the drawing, the electrical conductor preferably comprises a central core 10 of copper or similar conducting material 100 about which a plurality of conducting strands 11—11 are wrapped with a spiral lay in such a manner as to provide a smooth exterior surface. The exterior of this conductor as at 13 is roughened by rubbing with 105 an abrasive, such as sandpaper, or by subjecting it to the action of a sand blast. About the roughened surface 13 is closely wrapped the magnetic loading tape 12 which preferably consists of an alloy containing 78½% 110 nickel and 21½% iron.

After the composite conductor is provided with one or more layers of magnetic tape applied sufficiently tightly to make a good mechanical structure, the resulting conductor is 115 treated by passing it through a heated tubular furnace of the type disclosed in Fig. 2. This furnace which is of the muffled type comprises heating elements 30 which are located between the fire-clay muffle 31 and the 120 fire brick 32. The iron tube 33 has a copper lining 34 of such small inside diameter as to prevent rapid circulation of air which might cause an objectionable degree of oxidation of the magnetic tape. For the sake 125 of clearness, this apparatus has been shown schematically, but reference is made to an application of F. S. Kochendorfer, Serial No. 601,021, filed November 15, 1922 which has issued as Patent No. 1,624,668 on April 12, 130

1927 and which discloses the preferred form of apparatus to be used.

By providing an imperfect contact between the central conductor and the loading tape as is done by roughening one of the surfaces, the trouble due to adhesion formerly experienced has been largely overcome resulting in an improved conductor because of the higher permeability of the loading material. It is believed that this improved result is due to the fact that when the surfaces are roughened, the points of contact between the conductor and tape are of very small area; and although welding takes place at these points, these welds are readily broken up on contraction of the copper conductor without impressing undue strains on the magnetic tape. It is further possible that the cleaning of the conductor surfaces and the consequent removal of sulphides and other materials from the surface are partly instrumental in reducing the adhesion between the loading material and the conductor. Although it is preferable to roughen the surface of the conducting member because of its mechanical nature, an imperfect contact can also be obtained by roughening the under-surface of the tape.

What is claimed is:

1. A loaded signaling conductor comprising a central conductor having a rough, exterior surface, and a magnetic loading material wrapped closely about the rough surface, said loading material requiring heat treatment to develop high permeability therein, and the permeability of which is sensitive to strain, said rough exterior surface contacting with said loading material at a large number of closely spaced areas, thereby preventing the loading material from welding securely to said surface during the heat treatment.

2. A loaded signaling conductor comprising a central conductor having a cylindrical exterior surface roughened as by an abrasive, and a magnetic loading material wrapped closely about the rough surface, said loading material requiring heat treatment to develop high permeability therein, and the permeability of which is sensitive to strain.

3. A loaded signaling conductor comprising a central conductor having a cylindrical exterior surface roughened as by an abrasive, and a magnetic loading material wrapped closely about the roughened conductor, said loading material comprising a nickel iron alloy in which the nickel component predominates.

4. A loaded signaling conductor comprising a central conductor having a cylindrical exterior surface roughened as by an abrasive, and a magnetic loading material wrapped closely about the roughened conductor, said

loading material containing 78½% nickel and 21½% iron.

5. In a method of constructing a continuously loaded conductor having a cylindrical conducting portion and a magnetizable portion forming a layer wrapped in close contact with said conducting portion and which requires heat treatment to improve one of its electrical characteristics, the step of roughening the contacting surface of one of said portions to reduce deleterious interaction between said portions during said heat treatment.

6. The method of constructing a continuously loaded conductor which comprises roughening the surface of the conducting member by rubbing with an abrasive, wrapping a layer of magnetic material closely about the conducting member, and heat treating the loaded conductor.

7. A loaded signaling conductor comprising a conducting member having an outer surface and a magnetic member wrapped thereabout having an inner surface in close contact with said outer surface, one of said surfaces being roughened to form a large number of sharp closely spaced areas of contacts with the other of said surfaces thereby preventing the magnetic member from welding to said outer surface.

8. A loaded signaling conductor comprising a central conducting member and a magnetic loading material wrapped in close contact with said conducting member, said conducting member having a continuously interrupted outer surface for supporting said loading material by a large number of sharp, closely spaced contacts, thereby preventing the loading material from welding securely to said surface during the heat treatment.

9. A loaded signaling conductor comprising a central conducting member, a magnetic loading material wrapped in close contact with said conducting member, and means integral with the surface of one of the contacting elements for preventing the conducting member and loading material from securely welding to each other during heat treatment of the loaded conductor.

10. A loaded signaling conductor as described in claim 9 in which said means comprises a roughened surface on one of said contacting elements.

11. A loaded signaling conductor as described in claim 9 in which the magnetic material has a permeability sensitive to mechanical strain.

In witness whereof, I hereunto subscribe my name this 24th day of February, A. D. 1925.

JESSE F. WENTZ.

125

130